

Jan. 10, 1928.

1,655,507

C. A. NASH

ARTICLES HAVING POLISHED SURFACES

Filed July 1, 1921



INVENTOR.  
*Clarence A. Nash*  
BY *Franklin Hubbard*  
ATTORNEY

## UNITED STATES PATENT OFFICE.

CLARENCE A. NASH, OF MILWAUKEE, WISCONSIN, ASSIGNOR TO THE CUTLER-HAMMER MFG. CO., OF MILWAUKEE, WISCONSIN, A CORPORATION OF WISCONSIN.

## ARTICLES HAVING POLISHED SURFACES.

Application filed July 1, 1921. Serial No. 481,748.

This invention relates to articles having polished surfaces, particularly articles formed of plastic compositions, and to a method of constructing or producing articles having surfaces so polished.

Many articles, particularly those formed of plastic compositions as, for example, the insulating parts of various electrical devices, require a finish and high polish. However, such plastic compositions, especially when molded and subjected to a heat treatment are very difficult to finish as desired which characteristic has led to the use of surface coatings adapted to take a better finish but such coatings as heretofore treated have not proven entirely satisfactory.

The present invention has among its objects that of providing an article so constructed as greatly to facilitate the desired finish thereof.

Another object is that of providing articles so constructed as to materially improve the lustre, density and water resistivity of the finished surfaces thereof.

Another object is that of providing a simple and expeditious method of constructing articles having surfaces which exhibit the foregoing characteristics.

Other objects and advantages will herein-  
30 after appear.

According to the present invention it is proposed to construct the article with a surface layer of fusible material to be subjected to both a heat treatment and a smoothing and polishing treatment.

Preferably the article so constituted is subjected to a heat treatment preferably after partial buffing thereof. The temperature to which the aforementioned article is so subjected preferably substantially equals or somewhat exceeds that at which the fusible surface layer is adapted to soften, it having been found that the surface of the coating may thereafter be re-polished to produce a finish superior in brilliancy, durability and water resistivity to that obtainable by usual methods.

Referring to the accompanying drawing which illustrates one embodiment of the invention, the same shows an attachment plug cap comprising a molded insulating body 1 and a surface layer 2.

The body 1 may comprise any preferred composition such for example as the well known composition including a comminuted

asbestos filler and pitch binder. In practice such a base is commonly cold molded while plastic and baked until rendered very hard, the resultant product being inadapted to take a satisfactory finish.

The surface layer 2 may comprise any one of numerous fusible plastic compositions as for example one composed of coal tar pitch, substantially 60 parts, and finely divided silica or flint, substantially 40 parts. The proportions may vary between somewhat wide limits and are also influenced by the character of the finish desired, whereas numerous other substances or compounds may be employed as finishing material for such or other classes of pieces.

As a specific example of the instant method the following steps may be mentioned.

A body composed of a base material such as that described is treated to provide the same with a fusible surface layer of material such as that mentioned, which treatment may be effected preferably by buffing. In practice the material for such surface layer is preferably or conveniently applied directly to the surface of the buffing wheel or other smoothing device employed and thence transferred to the surface of the piece during the buffing or smoothing operation.

Such operation is preferably continued until a reasonably smooth and glossy exterior surface is obtained. The piece, having the fusible surface layer thus formed thereon, is thereafter subjected to heat treatment at a temperature preferably approximating or somewhat higher than that at which fusion of the surface layer or of the more readily fusible surface portions thereof, takes place.

The duration of such heat treatment may vary from somewhat less than half an hour to two hours or longer, dependent upon the size and shape of the piece and the character and consistency of the surface material thereof. It is also desirable that such treatment be continued long enough to effect thorough softening of the surface material without causing the latter to run, whereas, obviously such treatment should not be so long continued, or carried out at such temperature, as to injure the base material. Following such treatment the piece is permitted to cool sufficiently to effect setting or hardening of the surface material and is thereafter again polished either while still somewhat warm or at ordinary temperature. Such second

60

65

70

75

80

85

90

95

100

105

110

polishing operation is preferably effected also by buffing, the surface employed being preferably somewhat softer and more yielding than that employed during the first operation.

Such second polishing operation may be effected either with or without addition of a fresh surface material but in either case if the same instrumentality be employed for 10 several pieces consecutively its surface will ordinarily become to some extent covered or impregnated with such material.

The finish of pieces subjected to the complete treatment aforescribed is found to be 15 superior to that of pieces polished only by ordinary methods in the aforementioned respects among others.

A surface material such as that aforescribed is adapted to soften at a temperature 20 of approximately 180° to 200° F., dependent upon the constituency of the coal tar pitch employed, and the heat treatment where such compound is employed should be carried out preferably at a temperature 25 which may vary between 180° and 250° F. However, such temperature should preferably be high enough to effect softening and substantial fusion of the surface material, or of its more readily fusible constituents 30 without causing the latter to run off or separate from the base material.

Without limitation to any particular theory in accounting for the very marked improvements resulting from the aforescribed process of construction, it is believed 35 that where coal tar pitch or an analogous composite substance is employed as one of the principal constituents of surface material such coal tar pitch undergoes distillation 40 during the heat treatment, the more volatile constituents thereof being driven off leaving a residue which is much harder and denser and hence better adapted to receive and retain a high finish than is the material prior 45 to such treatment. Further it is believed that during the first smoothing operation the surface material is forced into more or less intimate contact with the base material to be covered thereby and also to some extent into any depressions or inequalities 50 which may exist in the surface of such material whereas during the heat treatment and consequent softening of the material constituting the surface layer the same is adapted to effect a more thorough amalgamation 55 with or impregnation of such surface, the relatively fluid state of the material obviously enabling the latter to penetrate the pores of the body as well as fill all depressions or minute cavities in the surface thereof, whereby the tenacity of adhesion of the 60 coating is greatly augmented. Also during such softening of the surface material the same tends to become covered with an exceedingly smooth film of its own substance,

due probably to the high surface tension of the softened material, which smoothness remains after cooling and consequent hardening, whereas the final polishing treatment should be so effected as not to remove or 70 impair such characteristic of the surface.

Thus, as a result of the aforescribed construction the articles produced thereby are characterized by exceedingly close and firm amalgamation of the surface material 75 as compared with similar pieces polished only by ordinary methods. Also the final finish of pieces produced as herein set forth is markedly superior in brilliancy, water resistivity and permanence to pieces produced 80 by ordinary methods.

It is, of course, to be understood that deviations from the aforesaid method may be made without departing from the scope of 85 the appended claims.

What I claim as new and desire to secure by Letters Patent is:

1. As an article of manufacture, a molded body of plastic composition having applied thereon a thermoplastic material comprising 90 a comminuted filler in suspension in a viscous binder, and adapted to be fused and reset in situ.

2. The method of polishing surfaces of 95 plastic composition articles, by impregnating with a fusible material and smoothing, which comprises application of said material by buffing and, as an intermediate distinct step, heat softening of the surface material undergoing treatment.

3. The method of polishing surfaces of 100 plastic composition articles, by impregnating with a fusible material and smoothing, which comprises, application of said material by buffing and, as a distinct step, heat softening with subsequent resetting of the surface material in situ prior to final smoothing thereof.

4. The method of constructing articles 105 having polished surfaces, which comprises providing the same with a surface layer of thermoplastic material which is capable of heat hardening, thereafter softening the surface material by application of heat, continuing the heat treatment for effecting volatilization and expulsion of constituents of the material to thereby increase the hardness of such material when cold, terminating the heat treatment to provide for setting of 110 the surface coating, and polishing the latter.

5. The method of constructing articles 115 having polished surfaces, which comprises providing the article with a surface layer of a fusible material capable of heat hardening, smoothing the exterior surface of such material, subjecting the article including such surface layer to heat treatment for thorough amalgamation of the surface layer with the body of the article and also for fusion and ultimate hardening of the surface material 120 125 130

and thereafter again smoothing the surface of such material.

6. The method of constructing articles having polished surfaces, which comprises forming upon the piece a surface layer of plastic finishing material having volatile constituents and smoothing the surface of such material, heating the article to effect amalgamation of said surface layer therewith and to expel certain of the volatile constituents of said surface material for hardening the residuum, and smoothing the surface of the material so hardened.

7. The method of constructing an article having a smooth surface of fine texture, which comprises applying to a cold molded and baked article of plastic material a surface layer of coal tar pitch and a finely di-

vided relatively infusible substance, and thereafter heating said surface layer to amalgamate it with the article to increase the surface density thereof.

8. The method of providing a smooth and dense surface on a cold molded and baked article of plastic composition, which comprises applying to said article by buffing a layer of coal tar pitch and finely divided silica, thereafter heating said article to effect amalgamation of said layer with the surface of said article and densification of the latter, and then further buffing or polishing said surface.

In witness whereof, I have hereunto subscribed my name.

CLARENCE A. NASH.